

Oct. 7, 1947.

S. J. EVERETT

2,428,518

HYPODERMIC TUBING, DENTAL BROACHES AND THE LIKE

Filed Dec. 31, 1943

FIG. 1.



FIG. 2A.



FIG. 2B.



FIG. 3.



FIG. 4.



FIG. 5.

Inventor

SAMUEL JAMES EVERETT,

By

Robert B. Parsons Attorney

## UNITED STATES PATENT OFFICE

2,428,518

HYPODERMIC TUBING, DENTAL BROACHES,  
AND THE LIKE

Samuel James Everett, Thornton Heath, England

Application December 31, 1943, Serial No. 516,573  
In Great Britain January 1, 1943

7 Claims. (Cl. 128—221)

1

This invention relates to fine metal articles, such as hypodermic needles, dental broaches and the like, and to a method of manufacturing the same.

One of the disadvantages of articles of this type is that having relatively fine diameters and being subjected to bending stresses during use, they are sometimes broken, thus causing injury to the patient. The broken off pieces frequently become lodged in body tissue and being small are sometimes lost or difficult of extraction.

In accordance with the present invention such articles are provided with a fibrous structure with the fibers being disposed predominantly transversely to the radius on which the bending takes place.

Where the article for example is a hypodermic needle, the crystalline structure of the needle is analogous to cane or bamboo with the fibrous structure being disposed predominantly longitudinally of the needle. A hypodermic needle so constructed resists breaking into two separate and distinct portions to a greater degree. Severe bending of the article may cause the needle to split longitudinally, but breakage into two separate parts is most difficult.

In the example of the hypodermic needle, if the needle is bent severely during usage, the fibers on the outer radius may break but the inner fibers split from the adjacent fibers so that the inner fibers bend on an easy or substantial radius such that they remain intact. There is, therefore, substantially no risk of the needle snapping into two separate and distinct parts. If the needle then breaks while in body tissue, there is no risk of the broken part becoming lost in the body.

It is a general object of the invention to provide fine metal articles such as hypodermic needles, tubing, dental broaches, surgical instruments, and the like, which possess this characteristic.

The invention has for another object the provision of fine metal articles of austenitic nickel-chromium steel, the crystalline structure of which is disposed predominantly in one direction, preferably at right angles to the radius on which the bending takes place.

These and other objects of the invention will become more apparent from the following description and claims when read in conjunction with the accompanying drawings in which:

Figure 1 is a diagrammatic representation of a section taken through the end of a hypodermic needle embodying the invention.

2

Figure 2A is a similar view showing a fracture resulting from severe bending stresses in a needle not embodying the invention.

Figure 2B is a similar view showing a fracture resulting from severe bending stresses in a needle embodying the invention.

Figure 3 is a diagrammatic view of part of a broken dental tool embodying the invention, and

Figures 4 and 5 are cross-sections, respectively, showing diagrammatically, billets used in the manufacture of further implements in accordance with the invention.

Figure 1 illustrates graphically the application of the invention to hypodermic needles. In the figure a portion of such a needle 1 is illustrated in cross section. The article is constructed preferably of austenitic nickel-chromium steel and for purposes of illustration the fibrous arrangement of the crystalline structure of the material is indicated in dash lines 2.

It will be noted that the fibrous arrangement is predominantly longitudinally of the needle which prevents the needle from breaking transversely into two separate pieces when subjected to bending stresses.

Figure 2A illustrates diagrammatically what happens when a needle 2, as hitherto manufactured, snaps as a result of severe bending. The metal at the outside of the bend parts at 2a while at 2b there is a sharp kink. Further bending will cause the needle to snap completely into two separate parts.

Figure 2B, on the other hand, shows what happens when a needle constructed according to the invention snaps as a result of severe bending. Again the metal at the outside of the bend snaps at 2a but the metal then splits longitudinally at 2c so that the metal at the inside of the bend is gently curved at 2d. Further bending will not substantially increase the radius of curvature at 2d and there is little risk of the metal breaking at 2d so that there is little risk of a part of the needle being left in the patient's body tissue. This property is due to the cane-like structure of the metal from which the needle is made.

Figure 3 is a diagrammatic section through a portion of a dental broach 3 according to the invention, the arrangement of the fibrous crystalline structure being indicated by the dash lines 4 bearing the reference numeral 4. When the broach is bent to such an extent that the fibers at the outside of the bend snap at 3a, longitudinal splitting takes place at 3c so that the fibers on the inside of the bend are on a long radius and the parts of the broach remain held together.

Articles such as have been described above may be produced in the following way: An austenitic nickel-chromium steel is first heated to about 1000° C. and is then cooled and cold-rolled, drawn or otherwise reduced in its cross sectional area by about 80% to 98%, depending upon the required cross section of the finished article. A length of such treated material is then further heated to eliminate internal stresses.

The temperature to which the metal is initially heated may be varied within certain limits. For example, instead of being heated to 1000° C., it may be heated for a somewhat longer time at 900° C., or heated for a shorter period at 1150° C., this being normal softening. The grain size can be controlled by the usual well known practice of quenching in oil or water.

The temperatures to which the final heating is carried in order to remove the stress or strain within the material may be varied but it is desired that this should be accomplished without destroying the fibrous structure which the material has at that time acquired. Thus, the article may be heated for a fairly long period at a temperature as low as 350° C., or for a shorter period as high as 475° C. In general, it may be said that experiments show that for most requirements the temperature should be about 400° C. for about two seconds for every one thousandth of an inch cross-sectional dimension, as for example, wall thickness of a tube or the diameter of a broach. If the heating is done at too low a temperature or too quickly, the required stability of the crystalline metallic structure is not obtained.

The type of austenitic nickel-chromium steel employed in making articles in accordance with the invention may vary within limits. However, the following is an example of the type of steel which can be employed advantageously: Firths' D. D. Q. steel containing 12% nickel and 12% chromium, the remainder being iron with traces of carbon and silicon. The steel should possess a high degree of resiliency and spring temper and great strength. Steels containing 18% nickel and 8% chromium can be cold worked to produce the required structure but are not so satisfactory in regard to their mechanical properties.

In producing fine tubing such as is employed in making hypodermic needles the following process is given by way of example: A billet of austenitic nickel-chromium steel is first drilled and by normal drawing process is then reduced until it has an outside diameter of approximately three sixteenths of an inch and a bore of approximately one-eighth of an inch. The tube is next annealed at 1000° C. and quenched. Then a one-eighth inch brass mandrel (70% copper, 30% zinc) is inserted, having first been lubricated by dipping in colloidal graphite. The brass rod is actually made about 0.008 inch smaller than the bore. The tube can then be cold drawn to 20 gauge, that is, 0.036 inch outside diameter. It is then straightened and heat treated at 400° C. for fifteen minutes to soften the brass mandrel and improve the structure of the steel. Finally, the tubing is divided into convenient lengths without, however, cutting the mandrel and the lengths are then drawn off the mandrel. The resulting lengths of tubing are found to have the longitudinal fibrous structure required. A similar method may be employed for the manufacture of dental broaches and similar fine steel instruments which are subjected to stresses approaching their ultimate strength, thereby eliminating the ever-pres-

ent danger of losing a portion of the instrument in the tissue of the body or cavity which is being operated upon.

It is, of course, a fact that the instrument when broken cannot always be pulled directly from the cavity or tissue, but the strong adherence of the broken part to the shank or remainder of the instrument enables the surgeon to make an incision in the correct place so that the parts can be successfully withdrawn.

In a modification of the aforesaid example, the initial billet, which may be half an inch to  $\frac{5}{8}$  inch in diameter, may comprise a sheath 8 of austenitic nickel-chromium steel over a tube 9 of stainless carbon steel, as shown in Figure 4. Heat treating at 1000° C., followed by air quenching softens the outer tube and hardens the inner one. An internal corrosion resisting lining 10 may be provided by providing inside the initial billet, a layer of nickel-silver, silver or nickel-chromium stainless steel. After the heat treatment, the composite billet is of course subjected to the extreme reduction in cross-section without further re-heating, as in the preceding example, to provide the austenitic nickel-chromium steel with the required fibrous or cane-like structure and thereby impart the required mechanical properties. To add to the fibrous structure high tensile wires 11 are embedded in the soft external sheath, the wires becoming integral with the tube wall during the extensive drawing operations. The final cane-like structure may also be enhanced by milling longitudinal slots in the initial billet.

As a variation of the methods just described, the fibrous structure of the tubing may be enhanced by building up the initial tubular billets from segments 12 (Figure 5) brazed together at their edges, the brazed joints 13 being not quite so strong as the segments themselves. If desired the segments can be composed of different metals.

Where the article is a dental broach or other similar structure of solid cross section, it may be made in accordance with the process first described from austenitic steel drawn down to a wire of the required size, the broach being formed from this wire before the final heating to remove the internal strain.

It will be understood that some changes may be made in the invention and that the description given in the accompanying illustrations are only to be considered as examples.

I claim:

1. An elongated surgical member of substantially reduced cross section and which is normally subjected during use to bending strains, said member being of austenitic nickel-chromium steel, the crystalline structure of the steel in the finished article being comprised of parallel elongated fibers disposed predominantly parallel to the longitudinal axis of said elongated member.

2. A surgical device or the like comprising an elongated thin steel body of cane-like fibrous structure comprised of longitudinally arranged elongated crystals, said longitudinally arranged elongated crystals being disposed substantially parallel to the longitudinal axis of said elongated steel body.

3. A surgical device or the like comprising an elongated austenitic nickel-chromium steel member of materially reduced cross section, said member having a predominantly longitudinal crystalline structure, ready to split longitudinally on bending.

4. A surgical device of austenitic nickel-chro-

mium steel, said device being elongated and having a reduced cross sectional diameter substantially equal to that of a 20 gauge wire, the crystalline structure of the finished device being made up of elongated fibers disposed predominantly longitudinally of the device, whereby said device will split longitudinally on bending.

5. A hypodermic needle of austenitic nickel-chromium steel, the crystalline structure of said needle being predominantly longitudinal, whereby said needle will split longitudinally on bending.

6. A hypodermic needle comprised of a tube of stainless carbon steel and a concentric outer sheath of austenitic nickel-chromium steel, rendered cane-like in structure by cold elongation in the direction of the axis of the needle.

7. A hypodermic needle comprising a tube of austenitic nickel-chromium steel rendered cane-like in structure by elongation in the cold state in the direction of the axis of said needle and a highly corrosion resistant layer on the inner surface of such tube.

SAMUEL JAMES EVERETT.

#### REFERENCES CITED

The following references are of record in the file of this patent:

#### UNITED STATES PATENTS

| Number     | Name     | Date          |
|------------|----------|---------------|
| 2,217,602  | Smith    | Oct. 8, 1940  |
| 2,208,606  | Smith    | July 23, 1940 |
| 2,041,778  | Peters   | May 26, 1936  |
| Re. 14,820 | Sallows  | Mar. 16, 1920 |
| 2,145,171  | Giles    | Jan. 24, 1939 |
| 2,187,259  | Barnhart | Jan. 16, 1940 |
| 2,217,602  | Smith    | Oct. 8, 1940  |
| 145,217    | Leiter   | Dec. 2, 1873  |
| 1,942,150  | Rohn     | Jan. 2, 1934  |

#### OTHER REFERENCES

- 20 Metallurgy & Metallurgical Engineering Series, "The Structure of Metals," C. S. Barrett, pp. 446 to 448.  
 Transactions American Society for Metals, vol. 23, Jan.-Dec. 1935, pp. 400-404.